# EUROPEAN PATENT SPECIFICATION

(11) **EP 4 493 644 B1**
(45) Date of publication and mention of the grant of the patent: **06.05.2026**
(21) Application number: 23728112.6
(22) Date of filing: 14.03.2023
(51) Int. Cl.: C10G 1/00, C10G 3/00

(54) **PROCESS FOR THE PRODUCTION OF BIO-OIL FROM LIGNOCELLULOSIC BIOMASS**
VERFAHREN ZUR HERSTELLUNG VON BIOÖL AUS LIGNOCELLULOSEHALTIGER BIOMASSE
PROCÉDÉ POUR LA PRODUCTION DE BIO-HUILE À PARTIR DE BIOMASSE LIGNOCELLULOSIQUE

(30) Priority: 14.03.2022 IT 202200004886
(43) Date of publication of application: 22.01.2025
(73) Proprietor: Thermolysys S.r.l., 71016 San Severo (FG) (IT)
(72) Inventor: QUATTROPANI, Mario, 6900 Lugano (CH); FUMAGALLI, Enrico Carlo, 6900 Paradiso (Lugano) (CH)
(74) Representative: PGA S.p.A.
(86) International application number: PCT/IB2023/052452
(87) International publication number: WO 2023/175493

(56) References cited:
- CN-A- 108 424 805
- US-A1- 2017 029 739
- US-A1- 2018 216 139
- US-A1- 2020 231 879

## Description

### Field of the invention

The present invention relates to a process and apparatus for the production of bio-oil and biofuels from lignocellulosic biomass, particularly lignocellulosic biomass consisting of or including agricultural waste.

### State of the Art.

As global demand for fuels and chemicals increases and oil stocks are depleting, ethanol fuel producers are increasingly looking beyond corn, potatoes and other starchy crops as biomass for ethanol fuel production.

Particularly promising is cellulosic biomass which is derived from low-cost and abundant feedstocks, can achieve high yields and enables the production of fuels with high octane and other properties. The use of lignocellulosic feedstocks, such as woody plants, prairie grass blends, agricultural wastes, allows for environmental and economic benefits. Compared with current sources of biofuels, these biomass feedstocks require fewer agricultural inputs than annual crops and can be grown even on marginal agricultural land.

Processes and plants for producing biofuels from lignocellulosic biomass are known. For example, US 2014/0121423 outlines a method for digesting cellulosic biomass in a glycerol solvent system in a hydro-thermal digestion unit to produce fuel blends. Sources of cellulosic biomass include: forest residues, agricultural residues, herbaceous material, woody materials.

US 2008/312346 outlines a method for preparing lignocellulosic biomass for slurry treatment and fuel production.

Also known is document US 2012/079760, which outlines a method for producing biodiesel from biomass in a reactor in which biomass is heated and mixed with a mixer using "super-heated" water as a solvent.

Document US2020231879A1 discloses a process of producing a distillate fuel from lignin including: preparing a biomass-derived lignin solvent, dissolving the lignin in the biomass-derived solvent and separating undissolved lignin and mineral matter to produce a syncrude.

Document US2017029739A1 discloses a preparation of low viscosity bio-oils from hydrothermal liquefaction (HTL) of lignocellulosic biomass in the presence of a crude glycerol and water mixture.

In this regard, the Applicant perceived the need to improve the known type processes for the production of bio-oil and biofuels from lignocellulosic biomass.

In particular, the Applicant perceived the need to improve the yield of known processes and the quality of the product(s) produced.

The Applicant particularly perceived the need to make the lignocellulosic biomass deconstruction process more efficient.

### Summary of the invention

The Applicant found that deconstructing lignocellulosic biomass with chemical catalysts and at low temperature allows the raw materials to be broken down into intermediates that can be more easily liquefied in a subsequent hydrothermal liquefaction step.

The invention relates to a process for producing bio-oil from lignocellulosic biomass according to the appended claims.

An apparatus for producing bio-oil from lignocellulosic biomass is also disclosed.

The Applicant has verified that the invention makes it possible to increase the process efficiency and the yield of bio-oil obtained from biomass compared to processes of the prior art.

The Applicant has also verified that the invention makes it possible to improve the quality of the bio-oil obtained compared to the processes of the prior art.

In particular, the Applicant has verified that low-temperature deconstruction (i.e. at the indicated temperatures) allows the hard and rigid structure of the plant cell wall, which includes the biological molecules cellulose, hemicellulose and lignin bound tightly together, to be broken down into intermediates.

Further features and advantages will be elucidated by the detailed description of a preferred, but not exclusive, embodiment of a process according to the present invention and of an apparatus for the production of bio-oil and biofuels from lignocellulosic biomass.

### Description of drawings

This description will be given below with reference to the set of drawings, provided for illustrative and non-limiting purposes only, in which:
▪ Figure 1 illustrates a flowchart of a process according to the invention;
▪ Figure 2 shows a schematic view of an apparatus for carrying out the process according to the invention;
▪ Figure 3 is an elevation view of a reactor that is part of the apparatus in Figure 2.

### Detailed description

Referring to Figure 1 attached herein, a process for producing bio-oil and biofuels from lignocellulosic biomass is schematically illustrated in the flowchart. An apparatus for producing bio-oil and biofuels from lignocellulosic biomass is labeled as a whole with reference number 1 in Figure 2 and is configured to implement the process in Figure 1. The apparatus 1 comprises a plurality of elements/machines/facilities that can also be placed/at different locations and used/at different times, as will be explained below.

In accordance with the process of the invention, an amount of lignocellulosic biomass (such as woody plants, prairie grass mixtures, agricultural wastes/scraps, such as corn waste, wheat straw and rice straw, paper and wood processing waste sugarcane waste) is delivered to a pretreatment site where, by means of chippers and/or shredders 2, also of a type known per se and illustrated only schematically in Figure 2, the amount of lignocellulosic biomass is shredded to a comminuted lignocellulosic biomass having the consistency almost of flour.

The amount of comminuted lignocellulosic biomass can then be stored in a warehouse 3 for a certain period of time so that it will dry in contact with the atmosphere and lose at least some relative humidity. Instead of being stored in the warehouse 3 or after spending a certain period of time in the warehouse 3, the comminuted lignocellulosic biomass can be treated with a drier 4 so as to give the biomass a desired relative humidity. For example, the drier 4 (which may also be of a type known per se) is of the hot-air type, that is, it is equipped with a heat source that heats the air mass to increase its evaporative power.

The amount (batch) of comminuted and dried lignocellulosic biomass is fed into a reactor 5 like the one shown in Figure 3.

Such a reactor 5 comprises a tank 6 (vessel) provided with an upper opening 7 for the introduction of the amount (batch) of lignocellulosic biomass. The upper opening 7 is sealable by means of a door and special gaskets, e.g., graphite Flat Gasket - 538C type. A shaft 8 of a mixer/scraper 9 passes through a passage made at the top of the tank 6 and is connected to a motor 10 arranged externally to the tank 6. For example, the mixer/scraper 9 is of the gate type. A distal end of the shaft 6, opposite to that engaged with motor 10, carries notched scraper blades 11. In addition, the aforementioned shaft 8 is hollow so as to confine a conduit internally. The conduit is connected to a receptacle outside the tank 6 and containing or configured to contain a chemical catalyst comprising a mixture of sulfuric acid (H₂SO₄) and hydrogen peroxide (H₂O₂).

The aforementioned conduit can also be connected with an additional receptacle outside the tank 6 and containing or configured to contain industrial waste glycerol. The aforementioned conduit terminates in a plurality of nozzles 12 (i.e., open ends of the conduit in the tank) carried by the shaft 8 and configured to alternately, i.e., at different times, feed chemical catalyst or glycerol into the tank 6 via pumps and/or valves arranged or operatively active on piping, not illustrated, connecting the aforementioned two receptacles with the shaft 8.

Alternatively, the conduit is connected only to the receptacle containing or configured to contain the chemical catalyst while the glycerol is fed through other conduits that terminate in the tank or through the top opening 7.

The tank 6 has a lower opening 13 that can be opened or closed via a respective valve and is connected to a cistern 14 (Figure 1) via an appropriate pipeline or directly to a distillation column 15, which may be known in itself and is not described in detail here.

A first coil 16 is arranged in tank 6. The first coil 16 contains or is configured to contain a first heat transfer fluid that is stable at high temperatures and is operationally connected to a high-temperature source, not shown and external to the tank 6. The function of the first coil 16 (heating element) is to feed heat into the tank 6 via the first heat transfer fluid, which takes it from the high-temperature source and gives it to the tank 6. For example, the first heat transfer fluid is DelcoTerm^{®} SODB, which is a eutectic mixture of diphenyl oxide and biphenyl, usable as a boiling-condensing heat transfer medium up to 750 °F (400 °C). With low vapor pressure, high thermal conductivity and oxidation stability, DelcoTerm^{®} SODB offers excellent heat transfer properties for long periods of operation at temperatures up to 400°C. Maximum heat transfer to the tank 6 and/or to the equipment allows the use of smaller pumps, valves and heating coils. In addition, such spent fluid can be disposed of through a variety of environmentally acceptable methods, such as waste oil recycling or heavy fuel combustion.

A second coil 17 is arranged in tank 6. The second coil 17 contains or is configured to contain a second heat transfer fluid and is operationally connected to a low-temperature source, not shown and external to the tank 6. The function of the second coil 17 (cooling element) is to remove heat from the tank 6 via the second heat transfer fluid, which draws heat from the tank 6 and transfers it to the low-temperature source. The second heat transfer fluid is, for example, water or a coolant.

A tube 18 housed in tank 6 is arranged parallel to the shaft 8 and is connected to a hydrogen source, such as a pressure cylinder, not shown and external to the tank 6. The tube 18 has one or more openings that flow into the tank 6. The tube 18 is configured to feed hydrogen into the tank 6 via valves arranged or operatively active on piping, not illustrated, connecting the hydrogen source with the tube 18.

The reactor 5 also comprises a pressure regulator 19 placed on top of the tank 6, a vacuum pump 20 connected to the tank 6 and at least one thermocouple 21 arranged in the tank 6.

The reactor 5 comprises a control unit 19, e.g., an electronic control unit operated by a PID (Proportional-Integral-Derivate) algorithm and operationally connected to the motor 10 of the mixer/scraper 9, to the pumps and/or valves placed on the piping connected to the receptacle for the chemical catalyst, to the pumps and/or valves placed on the piping connected to the receptacle for glycerol, to valves placed between the first coil 16 and the high-temperature source, to valves placed between the second coil 17 and the low-temperature source, to the pressure regulator 19, to the vacuum pump 20, to the thermocouple 21, to the valves placed between the hydrogen source and the tube 18, to the valve of the lower opening 13.

The tank 6 and also the other reactor elements 5, such as the first coil 16, the second coil 17, the mixer/scraper 9, and the tube 18, are made of an alloy resistant to highly acidic and corrosive environments under high temperature and pressure conditions, e.g., Hastelloy C-276.

The control unit CU is programmed and/or configured to control processes in the reactor 5, as shown below. Specifically, the control unit CU is configured to temperature programming and controlling using ramps, isotherms and thermal cycling.

The amount (batch) of comminuted and dried lignocellulosic biomass introduced into the tank 6 of the reactor 5 is first subjected to a deconstruction step, which consists of adding the chemical catalyst, i.e., sulfuric acid (H₂SO₄) e.g., in an amount between 1.8% and 4% and hydrogen peroxide (H₂O₂) e.g., in an amount between 0.5% and 1.5% and bring and maintain the resulting mixture at a deconstruction temperature between 40°C and 60°C for between 10 minutes and 20 minutes, i.e., sufficient to break down the raw materials into intermediates that can be more easily liquefied in the subsequent hydrothermal liquefaction step. The control unit CU receives signals from the thermocouple 12 and controls the valves of the first coil 16 and/or the second coil 17, the pressure regulator 19 and the valves/pumps located on the piping connected to the receptacle for the chemical catalyst to achieve the above.

Deconstruction opens up the physical structure of biomass cell walls, making sugar polymers, such as cellulose and hemicellulose, more accessible. These polymers are then chemically broken down into simple sugar building blocks during the subsequent hydrolysis process.

Once the aforementioned deconstruction has been achieved, industrial waste glycerol, for example, is added in an amount between 25 percent and 30 percent to the amount of deconstructed biomass contained in the tank 6 and the amount of deconstructed biomass mixed with glycerol is brought to pressures and temperatures that cause hydrothermal liquefaction.

For example, deconstructed biomass mixed with glycerol is brought to pressures between 60 bar and 80 bar and temperatures between 200 °C and 275 °C for a liquefaction time between 10 min and 60 min. The control unit CU receives signals from the thermocouple 12 and controls the valves of the first coil 16 and/or the second coil 17, the pressure regulator 19 and the valves/pumps located on the piping connected to the glycerol vessel so as to achieve the above. Hydrothermal liquefaction is usually implemented in a reaction environment with a pH between 1 and 14 and in the presence of solid-state salts with high corrosive action. The process uses glycerin as a solvent and takes advantage of the increase in temperature to optimize the solubility of nonpolar compounds. Hydrothermal liquefaction of biomass allows the solid bio-polymer structure to be broken down into totally liquid components. The steps of biomass decomposition during the hydrothermal process can be summarized as follows: at about 100 °C, the watersoluble part of the biomass disperses into glycerol and hydrolysis occurs above 150 °C. Meanwhile, the biomass polymers, such as cellulose and hemicellulose, disintegrate into their monomeric chains. At about 200 °C and 1 MPa, the solid biomass becomes slurry. Finally, at about 300 °C and 10 MPa, liquefaction occurs and the oily product (bio-oil) is obtained.

During deconstruction and/or liquefaction, the amount of lignocellulosic biomass is mixed by the mixer/scraper 9 actuated by the motor 10 through the electronic control unit CU.

At the end of hydrothermal liquefaction, oxygen and moisture are removed from the amount of liquefied biomass contained in tank 6 of reactor 5 until hydrogenated bio-oil is obtained. In fact, bio-oil has low oxygen content and low stability over time, so its removal is necessary to make it similar to crude oil.

For this purpose, the control unit CU controls the vacuum pump 20, which extracts gas, vapors and oxygen from the tank 6, and controls the valves located between the hydrogen source and the tube 18 to feed pressurized hydrogen into the tank 6, i.e., to perform high-pressure hydrodeoxygenation (HDO), while the mixer/scraper 9 continues mixing. In high-pressure hydrodeoxygenation (HDO), hydro-desulfurization (HDS) catalysts, such as cobalt MoS₂ / Al₂O₃, are also preferably used.

High-pressure hydrodeoxygenation (HDO) is a high-pressure operation through which hydrogen is used to extract oxygen from bio-oil, giving a high-quality petroleum product. In addition, high-pressure hydrogenation can prevent carbon deposition on the catalyst surface, which facilitates reactor operation 5.

The hydrogenated bio-oil is either extracted from the tank 6 through the lower opening 13 and stored in cistern 14 and later taken to the distillation column 15 or directly fed into the distillation column 15.

According to a variant of the process, instead of by high-pressure hydrodeoxygenation (HDO) performed in the reactor 5, the removal of oxygen and moisture from the liquefied biomass is implemented by fast catalytic pyrolysis with zeolites at atmospheric pressure. Therefore, according to this variant, the liquefied biomass is extracted from the reactor 5 at the end of hydrothermal liquefaction and sent to a subsequent tank configured to implement the aforementioned fast catalytic pyrolysis with zeolites. At the end of catalytic pyrolysis, the obtained bio-oil is stored in cistern 14 and/or sent to distillation column 15.

In distillation column 15, in a manner also known in itself, bio-oil is fractionated to obtain second-generation bio-fuels. Bio-oil is in fact a mixture that can be separated into fractions. The bio-oil to be distilled enters distillation column 15 and the distillation products are separated and exit distillation column 15. Distillation column 15 has outlets 21 at intervals along its vertical development so that multiple products having different boiling ranges can be taken by distilling a multicomponent feed stream. "Lighter" products with the lowest boiling points exit from the head 22 of the column and "heavier" products with the highest boiling points exit from the bottom 23.

### Items list

apparatus 1
chippers and/or shredders 2
warehouse 3
drier 4
reactor 5
tank 6
upper opening 7
shaft 8
mixer/scraper 9
motor 10
notched scraper blades 11
nozzles 12
lower opening 13
cistern 14
distillation column 15
first coil 16
second coil 17
tube 18
pressure regulator 19
vacuum pump 20
outlets 21
head 22
bottom 23
control unit CU

## Claims

1. Process for the production of bio-oil from lignocellulosic biomass, comprising the following steps:
a) comminuting an amount of lignocellulosic biomass;
b) deconstructing the amount of comminuted lignocellulosic biomass;
c) adding glycerol in mixing with the amount of deconstructed biomass;
d) bringing the amount of deconstructed biomass mixed with glycerol to pressures and temperatures that cause hydrothermal liquefaction;
e) removing oxygen and moisture from the liquefied amount of biomass until a hydrogenated bio-oil is obtained, wherein the removal of oxygen and moisture from the liquefied biomass is carried out by high-pressure hydrodeoxygenation (HDO) or by fast catalytic pyrolysis with zeolites;
wherein deconstructing the amount of lignocellulosic biomass comprises: adding at least one chemical catalyst and maintaining the amount of lignocellulosic biomass at a deconstruction temperature between 30°C and 90°C, until said lignocellulosic biomass is deconstructed.

2. Process according to claim 1, further comprising: treating hydrogenated bio-oil by fractional distillation until second-generation bio-fuels are obtained.

3. Process according to claim 1 or 2, wherein the amount of lignocellulosic biomass is comminuted until it becomes like flour, optionally through the use of chippers and/or shredders.

4. Process according to one of claims 1 to 3, wherein after shredding the amount of lignocellulosic biomass and before deconstructing it, the process comprises:
a') drying the amount of comminuted lignocellulosic biomass to remove at least some of the relative humidity.

5. Process according to one of claims 1 to 4, wherein said at least one chemical catalyst comprises a mixture of chemicals.

6. Process according to claim 5, wherein the mixture of chemicals comprises sulfuric acid (H₂SO₄) and hydrogen peroxide (H₂O₂).

7. Process according to claim 6, wherein the sulfuric acid (H₂SO₄) added in the amount of lignocellulosic biomass is in the range of 1.8% to 4%.

8. Process according to claim 6 or 7, wherein the hydrogen peroxide (H₂O₂) added in the amount of lignocellulosic biomass is in the range of 0.5% to 1.5%.

9. Process according to one of claims 1 to 8, wherein the glycerol added in mixing is industrial waste glycerol.

10. Process according to one of claims 1 to 9, wherein the glycerol is waste from desalinated glycerol.

11. Process according to one of claims 1 to 10, wherein, in order to cause hydrothermal liquefaction, the deconstructed biomass mixed with glycerol is raised to pressures between 50 bar and 100 bar and temperatures between 180 °C and 300 °C.

12. Process according to one of claims 1 to 11, wherein glycerol is added in the range of 25% to 30%.

13. Process according to one of claims 1 to 12, wherein the deconstruction temperature is between 40°C and 60°C.

14. Process according to one of claims 1 to 13, wherein the amount of lignocellulosic biomass is maintained at the deconstruction temperature for a deconstruction time between 10 minutes and 20 minutes.

15. Process according to one of claims 1 to 14, wherein the amount of deconstructed biomass mixed with glycerol is brought to the pressures and temperatures to cause hydrothermal liquefaction for a liquefaction time between 10 min and 60 min.

## Patentansprüche

1. Verfahren zur Herstellung eines Bio-Öls aus lignozellulosischer Biomasse, umfassend die folgenden Schritte:
a) Zerkleinern einer Menge lignozellulosischer Biomasse;
b) Aufschließen der Menge der zerkleinerten lignozellulosischen Biomasse;
c) Zugabe von Glycerin unter Vermischung mit der Menge der aufgeschlossenen Biomasse;
d) Bringen der Menge an aufgeschlossener und mit Glycerin vermischter Biomasse auf Drücke und Temperaturen, die eine hydrothermale Verflüssigung bewirken;
e) Entfernen von Sauerstoff und Feuchtigkeit aus der verflüssigten Menge an Biomasse, bis ein hydriertes Bio-Öl erhalten wird, wobei das Entfernen von Sauerstoff und Feuchtigkeit aus der verflüssigten Biomasse durch Hochdruck-Hydrodeoxygenierung (HDO) oder durch schnelle katalytische Pyrolyse mit Zeolithen durchgeführt wird;
und wobei das Aufschließen der Menge an lignozellulosischer Biomasse umfasst:
- die Zugabe mindestens eines chemischen Katalysators und
- das Halten der lignozellulosischen Biomasse bei einer Aufschlusstemperatur zwischen 30 °C und 90 °C, bis die lignozellulosische Biomasse aufgeschlossen ist.

2. Verfahren nach Anspruch 1, ferner umfassend:
Behandeln des hydrierten Bio-Öls durch fraktionierte Destillation, bis Biokraftstoffe der zweiten Generation erhalten werden.

3. Verfahren nach Anspruch 1 oder 2, wobei die Menge an lignozellulosischer Biomasse so zerkleinert wird, dass sie eine mehlartige Form annimmt, optional unter Verwendung von Häckslern und/oder Schreddern.

4. Verfahren nach einem der Ansprüche 1 bis 3, wobei das Verfahren nach dem Zerkleinern der Menge an lignozellulosischer Biomasse und vor deren Aufschluss umfasst:
a') Trocknen der Menge an zerkleinerter lignozellulosischer Biomasse, um zumindest einen Teil der relativen Feuchtigkeit zu entfernen.

5. Verfahren nach einem der Ansprüche 1 bis 4, wobei der zumindest eine chemische Katalysator eine Mischung von Chemikalien umfasst.

6. Verfahren nach Anspruch 5, wobei die Mischung von Chemikalien Schwefelsäure (H₂SO₄) und Wasserstoffperoxid (H₂O₂) umfasst.

7. Verfahren nach Anspruch 6, wobei die der Menge an lignozellulosischer Biomasse zugesetzte Schwefelsäure (H₂SO₄) in einem Bereich von 1,8 % bis 4 % liegt.

8. Verfahren nach Anspruch 6 oder 7, wobei das der Menge an lignozellulosischer Biomasse zugesetzte Wasserstoffperoxid (H₂O₂) in einem Bereich von 0,5 % bis 1,5 % liegt.

9. Verfahren nach einem der Ansprüche 1 bis 8, wobei das beim Vermischen zugesetzte Glycerin industrielles Abfallglycerin ist.

10. Verfahren nach einem der Ansprüche 1 bis 9, wobei das Glycerin Abfall aus entsalztem Glycerin ist.

11. Verfahren nach einem der Ansprüche 1 bis 10, wobei zur Bewirkung der hydrothermalen Verflüssigung die aufgeschlossene und mit Glycerin vermischte Biomasse auf Drücke zwischen 50 bar und 100 bar sowie Temperaturen zwischen 180 °C und 300 °C gebracht wird.

12. Verfahren nach einem der Ansprüche 1 bis 11, wobei Glycerin in einem Bereich von 25 % bis 30 % zugesetzt wird.

13. Verfahren nach einem der Ansprüche 1 bis 12, wobei die Aufschlusstemperatur zwischen 40 °C und 60 °C liegt.

14. Verfahren nach einem der Ansprüche 1 bis 13, wobei die Menge an lignozellulosischer Biomasse für eine Aufschlusszeit zwischen 10 Minuten und 20 Minuten bei der Aufschlusstemperatur gehalten wird.

15. Verfahren nach einem der Ansprüche 1 bis 14, wobei die Menge an aufgeschlossener und mit Glycerin vermischter Biomasse für eine Verflüssigungszeit zwischen 10 Minuten und 60 Minuten auf die Drücke und Temperaturen gebracht wird, die eine hydrothermale Verflüssigung bewirken.

## Revendications

1. Procédé de production de bio-huile à partir de biomasse lignocellulosique, comprenant les étapes suivantes consistant à :
a) finement hacher une quantité de biomasse lignocellulosique ;
b) déconstruire la quantité de biomasse lignocellulosique finement hachée ;
c) ajouter du glycérol par mélange avec la quantité de biomasse déconstruite ;
d) porter la quantité de biomasse déconstruite mélangée au glycérol à des pressions et à des températures qui entraînent une liquéfaction hydrothermique ;
e) retirer l'oxygène et l'humidité de la quantité liquéfiée de biomasse jusqu'à ce qu'une bio-huile hydrogénée soit obtenue, dans lequel le retrait de l'oxygène et de l'humidité de la biomasse liquéfiée est exécuté par hydrodésoxygénation sous haute pression (HDO) ou par pyrolyse catalytique rapide avec des zéolites ;
dans lequel la déconstruction de la quantité de la biomasse lignocellulosique comprend l'étape consistant à : ajouter au moins un catalyseur chimique et à maintenir la quantité de biomasse lignocellulosique à une température de déconstruction comprise entre 30°C et 90°C, jusqu'à ce que ladite biomasse lignocellulosique soit déconstruite.

2. Procédé selon la revendication 1, comprenant en outre l'étape consistant à : traiter la bio-huile hydrogénée par distillation fractionnée jusqu'à ce que des bio-carburants de seconde génération soient obtenus.

3. Procédé selon la revendication 1 ou 2, dans lequel la quantité de biomasse lignocellulosique est finement hachée jusqu'à ce qu'elle ressemble à de la farine, éventuellement à travers l'utilisation de déchiqueteuses et/ou de désintégrateurs.

4. Procédé selon l'une des revendications 1 à 3, dans lequel après la désintégration de la quantité de biomasse lignocellulosique et avant sa déconstruction, le procédé comprend l'étape consistant à :
a') sécher la quantité de biomasse lignocellulosique finement hachée pour retirer au moins une partie de l'humidité relative.

5. Procédé selon l'une des revendications 1 à 4, dans lequel ledit au moins un catalyseur chimique comprend un mélange d'agents chimiques.

6. Procédé selon la revendication 5, dans lequel le mélange d'agents chimiques comprend de l'acide sulfurique (H₂SO₄) et du peroxyde d'hydrogène (H₂O₂).

7. Procédé selon la revendication 6, dans lequel l'acide sulfurique (H₂SO₄) ajouté dans la quantité de biomasse lignocellulosique se situe dans la plage de 1,8 % à 4 %.

8. Procédé selon la revendication 6 ou 7, dans lequel le peroxyde d'hydrogène (H₂O₂) ajouté dans la quantité de biomasse lignocellulosique se situe dans la plage de 0,5 % à 1,5 %.

9. Procédé selon l'une des revendications 1 à 8, dans lequel le glycérol ajouté en mélange est du glycérol de déchets industriels.

10. Procédé selon l'une des revendications 1 à 9, dans lequel le glycérol est un déchet provenant de glycérol de dessalement.

11. Procédé selon l'une des revendications 1 à 10, dans lequel, afin d'amener la liquéfaction hydrothermique, la biomasse déconstruite mélangée au glycérol est élevée à des pressions comprises entre 50 bars et 100 bars et à des températures comprises entre 180°C et 300°C.

12. Procédé selon l'une des revendications 1 à 11, dans lequel le glycérol est ajouté dans la plage de 25 % à 30 %.

13. Procédé selon l'une des revendications 1 à 12, dans lequel la température de déconstruction est comprise entre 40°C et 60°C.

14. Procédé selon l'une des revendications 1 à 13, dans lequel la quantité de biomasse lignocellulosique est maintenue à la température de déconstruction sur une durée de déconstruction comprise entre 10 minutes et 20 minutes.

15. Procédé selon l'une des revendications 1 à 14, dans lequel la quantité de biomasse déconstruite mélangée au glycérol est portée à des pressions et à des températures conduisant à la liquéfaction hydrothermique sur une durée de liquéfaction comprise entre 10 min et 60 min.
